

Patented Nov. 14, 1944

2,362,884

# UNITED STATES PATENT OFFICE

2,362,884

## PROCESS OF MAKING ALUMINUM COATED PAPER

John W. Clark, Westbrook, Maine, assignor to  
S. D. Warren Company, Boston, Mass., a corporation of Massachusetts

No Drawing. Application April 9, 1941,  
Serial No. 387,778

1 Claim. (Cl. 117—71)

This invention relates to the provision of aluminum-coated web or sheet material, e. g., regenerated cellulose films, resinous films, and fibrous webs such as paper or textile webs. In particular it pertains to aluminum-coated sheet material in which the aluminum coating is deposited from an aqueous medium. The finished product has properties of glossiness and reflection of visible and/or infra-red radiation not possessed by previous aluminum-coated sheet material of the same general class.

Aluminum powder, both from the standpoint of original color and especially color after aging, has long been recognized as superior to powders of zinc, tin or other white metal (exclusive of the expensive noble metals) for use in making metallic coated or so-called "silver" papers. A large volume of fine quality aluminum-coated paper, having a mat or dull surface, is made annually. Generally speaking this production falls into two classes, i. e., so-called "lacquer-metallics" and "casein-metallics." The term "lacquer-metallics" is used to designate paper which is coated with a suspension of metal powder suspended in a cellulosic or resinous lacquer or varnish. Such coatings dry smooth, with a good sheen, but with low specular reflection. Lacquer metallics have usually been considered to be the best grade of aluminum-coated papers on the market. A cheaper grade of paper, the so-called "casein metallics" has been made by coating a paper base with an aqueous suspension of aluminum powder and a water-dispersible adhesive, such as casein. Such coatings usually do not dry smooth and so have to be treated, as by calendering, to remove cockle from the sheet. Such papers have been usually considered somewhat inferior to lacquer-metallic coated paper in appearance.

In both lacquer-metallic and casein-metallic coatings the metal powder and the binder are so mixed that the layer of coating is of similar composition throughout. It may be that "leafing" may take place to some extent—that is, that there may be a tendency for some of the metal flakes to rise to the top of the coating before the coating sets, so that there is a slightly higher concentration of metal at the surface than beneath the surface—but in any case the difference is slight, and for practical purposes the composition may be considered to be uniform throughout.

Some aluminum-coated papers of both the lacquer-metallic type and the casein-metallic type fairly well approximate the appearance of dull or unpolished aluminum foil. Prior to the present invention, however, no such aluminum-coated paper of either type has, so far as I know, even remotely approached polished aluminum foil in appearance. In fact the belief has been

quite general among paper-coaters that it was impossible to make an aluminum-coated paper of either the lacquer-metallic or casein-metallic type which would resemble polished foil in appearance.

The desirability of making an aluminum-coated paper resembling polished foil in appearance has long been apparent. Various methods of producing such paper have been suggested. One more or less successful method comprises spreading over a paper base a resinous composition and, while the resinous coat is tacky, dusting it with aluminum powder. The excess powder is then removed by a brush or other polishing device, leaving only the metal particles which actually contact the resinous coat. The coating is then preferably "cured" as by heating. It is apparent that such a coating, in contradistinction to the more or less homogeneous coatings of the lacquer-metallic and casein-metallic types, is composed of two distinct layers, i. e., a layer of resinous binding material next to the paper, with a thin surface layer of metal flakes lying thereon. The lower side of each flake is anchored in the resin while the top side is exposed substantially free from any covering material. As a result, when properly burnished such coated paper may exhibit a polished aluminum surface which approaches polished foil in appearance. Such paper reflects visible light very well, but owing to the comparative thinness of the metallic layer it would not be expected that the more penetrating infra-red rays would be reflected so well; actually the most attractive of the products of this type with which I am familiar is known to have poor heat reflective properties, i. e., to have a high emissivity value.

The product of the present invention is an aluminum-coated sheet material which, contrary to prior aluminum-coated papers, has a low heat emissivity value, in the order of 0.2 or less, preferably in the order of about 0.1 or less. The product has a coating which is substantially uniform throughout, being deposited from a liquid slurry in which aluminum powder is thoroughly mixed with an aqueous binding material. Moreover the product has to a considerable degree the appearance of polished aluminum foil. The degree of resemblance of the product to polished foil and its difference from prior aluminum-coated papers having coatings deposited from aqueous media are easily apparent to the eye. In some cases the product of the invention may hardly be distinguished from polished foil in appearance, while in all other cases the appearance of my product is much nearer to that of polished foil than has been attained by prior coated paper having water-deposited aluminum coatings.

There is not, to my knowledge, any absolute measure of "polished metallic appearance." However, polished metal and other very shiny surfaces are distinguished by certain optical characteristics which, while having no absolute correlation with polished metallic appearance, are nevertheless definitely not possessed by material having no shiny appearance. Of the measurements of (1) "specular gloss," (2) "luminous apparent reflectance" and (3) "apparent-reflectance contrast," each affords means of scientific definition of certain such optical characteristics which go with polished metallic appearance. Without at present going into detail as to the nature of the aforementioned measurements it will suffice to state that my products have a specular gloss of at least 25, while prior casein-aluminum coated papers have not had a specular gloss in excess of about 10. The products of my invention likewise have a luminous apparent reflectance of not over 0.20, whereas prior "casein-metallic" papers (aluminum) have shown values of about .35 to about .30. The apparent-reflectance contrast value of my products is 100 or more, while that of prior casein-aluminum paper has been not over about 25.

The considerable difference in gloss properties between my product and prior casein-aluminum coated papers indicates that either the proportions of coating ingredients used for my product have not been used before or that the particular finishing methods I use have not been applied to previous casein-aluminum papers, or both.

To make the product of the present invention an aqueous suspension is prepared comprising aluminum powder and suitable water-dispersible adhesive, the proportion of adhesive to aluminum powder being notably less than in similar water-dispersible adhesive-aluminum compositions heretofore used for paper coating whereby to provide an adhesive-aluminum coating which is definitely "slack-sized" as contrasted with prior art, conventional, casein-aluminum coatings; the suspension slurry is applied to a suitable flexible web such as a web of paper; the coated web is dried; and then the coating is smoothed by heavy rolling pressure. If desired, the smoothed coated surface may subsequently be burnished, buffed, or otherwise polished.

The base stock to which the aluminum coating is applied may be a paper, textile, regenerated cellulose web or the like. When paper is used as the base, it may be calendered or supercalendered; or preferably the base may be a paper or a textile web bearing on its surface a layer of mineral coating (e. g., clay or other pigment and adhesive such as starch, casein or the like), which mineral-coated surface may, if desired, be calendered and/or supercalendered. Superior results are obtained by use of a base stock carrying a relatively heavy mineral coating, e. g., a coating of over 15 pounds per ream on one side. In some cases it is advantageous to have the surface of the base stock and/or the mineral coating colored or dyed to approximately the color of the aluminum coating applied thereto: such color in the underlying surface makes possible the use of a thin layer of metallic coating without danger of the base stock being discernible through the metallic coating when the product is complete.

The aqueous slurries of aluminum powder and adhesive may be applied to the base stock by any conventional coating means, such as a brush, knife-blade, roll, or spray-gun. A preferred method is the well-known air-blade or "air-

brush" method disclosed by Lebel in U. S. Patent No. 1,980,923.

Adhesives suitable for use in preparing aqueous slurries of aluminum powder in accordance with the present invention include various materials soluble in water or dilute alkali, including: carbohydrates, such as starch; proteins, such as glue, casein, and soy bean protein; and water-soluble resinous substances, such as polyvinyl alcohol, "Petrox" resin, and the like. Because of its efficiency and relatively low cost, casein is expedient to use. In using casein, care should be exercised to use no large excess of alkali for dissolving the casein, because a large excess of alkali may act adversely by dissolving part of the aluminum powder.

Any of the various aluminum or aluminum bronze powders commonly used in the manufacture of aluminum coated papers are usable in the carrying out of the invention. Commercial aluminum powders are supplied in various grades such as "litho," "standard," "extra brilliant," "lining," "extra fine lining," etc. Commercial aluminum powders are prepared by the use of hammermills, or similar devices, and during the process of manufacture they are coated with more or less grease of some kind. For my purpose, the less grease on the powder the better. In any case, however, it is advisable, before preparing the aqueous coating mixture, to wet the metal powder with a wetting agent, such as an alcohol, a sulphonated naphthalene derivative, a sulphate of a high aliphatic alcohol, or the like; such wetting materially assists in obtaining good dispersion of the powder in the aqueous mixture and insures contact being made between the metallic particles and the adhesive.

It will be readily understood that variations in particle size, surface area, and other properties of the aluminum powder particles, as well as in quantity of grease upon them, will cause variations in the adhesive requirement among different powders. The adhesive requirement may be understood to be the least quantity of adhesive which will bind a unit quantity of the metal powder satisfactorily in the use to which the coating is to be put. Since the adhesive requirement varies depending upon the properties of the aluminum powder used and also to some extent upon the particular base stock used, it is apparent that no fixed ratio of adhesive to metal powder can be set as optimum. Generally speaking, the best results in respect to finish and metallic appearance result when the ratio of adhesive to aluminum is kept as low as possible. I prefer to use not over 35 parts by weight of adhesive to 100 parts of aluminum powder and I usually obtain better results if I use less than 35 parts, say 25 or 30 parts, of adhesive to 100 parts of aluminum powder. Of course, it is to be understood that the finish, gloss, or metallic appearance of the product depend not alone on the adhesive-metal ratio, but also upon the finishing treatment given the coated web. For instance, a coating containing not over 35 parts of adhesive to 100 of aluminum may be calendered moderately to show a specular gloss of say 25 and thus fall within the limits of my acceptable products, or it may be treated further according to my preferred buffing treatment (to be described hereinafter) to acquire a considerably higher gloss. On the other hand, a coating containing a higher ratio of adhesive to aluminum, say, 40 or 45 to 100, almost certainly will not, when merely calendered, take a gloss sufficiently high to fall with-

in the scope of my invention; but such a coating when further treated according to my preferred buffing process may attain a gloss high enough to bring it within the lower limits acceptable for my product. Even 45 parts of adhesive to 100 parts of aluminum is considerably less than it has been customary to use in previous casein-aluminum coatings, however: for example, the coating of a typical, high grade, commercial "silver" paper was found to contain 72 parts of casein to 100 parts of aluminum powder. On the other hand, as previously stated, I prefer not to use more than 35 parts of adhesive to 100 of aluminum, i. e., not more than approximately half the quantity that has been used in typical prior aluminum coated paper. Usually I need to use less than 35 parts, say from 20 to 30 parts of adhesive. I have successfully used as little as 15 parts of casein, or correspondingly small amounts of other water-dispersible adhesives, to 100 parts of aluminum powder.

The paper coated with aqueous aluminum powder slurry as hereinbefore described may be dried in any usual manner, as by currents of hot air, on sticks, or against internally heated drying surfaces. The dried paper is then subjected to relatively heavy pressure to smooth the coating. The smoothing means may suitably be a calender stack of all metal rolls, or a supercalender comprising alternate metal and softer rolls, or a friction-calender having a driven friction-roll running at a speed different from the paper speed, or any combination of such calenders, depending upon the exact type of finish desired. The heavy rolling pressure exerted by the calender acts to align the particles and press them together so that they present substantially a single plane surface more or less closely resembling that of sheet metal. Calendering the sheet while the coated surface is moist is advantageous in order to increase the flatness of surface; very heavy moistening of the sheet is permissible. The use of polished calender rolls is advantageous to increase the smoothness and gloss of the calendered surface. The method and apparatus disclosed for supercalendering varnishable printing paper in Cates U. S. Patent No. 2,088,893 are very suitable for use to make the present product. Heavy calendering of some sort is a practical essential in the production of my improved product.

If desired, the calendered sheet may be further treated to increase the polish and specular reflection of the surface. Polishing or burnishing devices, such as brushes or cloth buffering rolls, may be used, or methods such as those commonly employed in polishing metal foil may be resorted to. In carrying out the buffering operation I have found it advantageous to use a polishing agent on the buffering roll or rolls: the polishing agent should, naturally, be in an extremely finely divided state. For this purpose fine grades of silicious powder, emery powder, polishing rouge, tripoli, and finely divided chromium oxide have been used with success, particularly when mixed with a small quantity of waxy, resinous, or other suitable binder. The process of buffering is generally described and claimed in my co-pending application filed July 12, 1939, Serial No. 284,088, entitled "Paper with improved surface." Apparently a real grinding or polishing action is obtained when such polishing agents are employed in the buffering. Whatever the finishing process employed, however, the finished product exhibits an appearance more like that of true metal foil

than is obtained by applying the same finishing operations to previous papers having coatings deposited from aqueous suspensions of aluminum and adhesive in which the conventional ratios of adhesive to metal powder have been adhered to.

The effect of polishing ordinary "casein metallics" with a buffering roll and abrasive is usually to raise the gloss appreciably; but no great improvement in actual metallic appearance results. In the case of my product, however, the effect of the buffering treatment is striking; the buffed product closely resembles highly polished metal foil in appearance, and its specular reflection is so greatly increased that, generally speaking, the gloss of the product can not be measured on the Bausch & Lomb Glossmeter, a standard instrument for measuring gloss of customary glossy papers. Hence, it is apparent that results are attained by buffering my product which have not been even closely approached by previous casein-aluminum coated papers.

The following examples, in which the "parts" are parts by weight, are given to show some specific coating compositions suitable for use according to the invention:

#### Example 1

|                                          | Parts |
|------------------------------------------|-------|
| Aluminum powder, litho grade             | 100   |
| Butanol (wetting agent)                  | 20    |
| 30 Casein dissolved by alkali (adhesive) | 20    |
| Water                                    | 200   |

#### Example 2

|                                                                  | Parts |
|------------------------------------------------------------------|-------|
| 35 Aluminum powder, extra fine litho grade                       | 100   |
| "Aerosol," a sulphonate of a dioctyl malic ester (wetting agent) | 1     |
| Soy bean protein dissolved by alkali (adhesive)                  | 25    |
| 40 Water                                                         | 250   |

#### Example 3

|                                              | Parts |
|----------------------------------------------|-------|
| Aluminum powder, extra brilliant litho grade | 100   |
| 45 Turkey-red oil (wetting agent)            | 5     |
| Oxidized corn starch (adhesive)              | 35    |
| Water                                        | 250   |

#### Example 4

|                                  | Parts |
|----------------------------------|-------|
| 50 Aluminum powder, lining grade | 100   |
| Butanol                          | 20    |
| Polyvinyl alcohol (adhesive)     | 15    |
| Water                            | 175   |

55 Following is a description of the preferred manner of carrying out the process of the invention:

For the base there is selected a mineral-coated paper of which the uncoated body stock amounts to about 50 pounds per ream (of 500 sheets cut to 25 x 38 inches) and which has on one side a mineral coating of from 13 to 20 pounds, the mineral coating comprising inorganic pigment such as clay, calcium carbonate and the like, and adhesive such as casein, starch and the like. To the coated side of the base paper is applied, by means of an "air-brush" coating machine, from 5 pounds to 1 pound, or even less, dry weight, of an aqueous aluminum coating composition similar to preceding Example 1, or any other of the examples previously cited. The coated paper is dried by any conventional method, preferably by the passage thereover of hot air currents. The coated and dried sheet is then—preferably after being moistened (e. g., steamed) heavily on the coated side—run through a stack of calendar rolls in

which hard or metal rolls contact the coated side of the paper. Preferably the hard rolls contacting the coated sheet have highly polished surfaces; the other rolls of the stack may be either metal or fiber rolls, but in any case relatively hard rolls are preferred. The calendering preferably is conducted under heavy pressure, suitably the heaviest pressure which the coated paper will bear.

If the treatment be stopped at this point, i. e., after the calendering operation, it will be found that the product is of excellent appearance, and has a gloss considerably higher than that hitherto known in aluminum coated papers coated from aqueous suspension, and higher than that of dull or unpolished aluminum foil. If a higher gloss is desired, the calendered paper may be further treated by subjecting it to the action of one or more buffing rolls used in conjunction with suitable fine abrasive powder as previously described. Such buffing rolls have not prior to my invention, to my knowledge, been used in the treatment of paper. Such rolls have a soft yieldable surface, such as fabric. The buffing roll or rolls revolve at high speed while contacting the sheet, which may be held against the buffing roll by a supporting roll. As a result of the buffing action the luster of the aluminum-coated surface is increased until it practically equals or even surpasses that of usual grades of polished aluminum foil.

The calendered, or calendered and buffed, product may, if desired, be embossed by known means, to provide a desired embossed effect.

It should be noted that in case colored coatings are desired, colored aluminum powders may be employed in the coating compositions. Or one may use uncolored aluminum powder, but color the coating compositions by dyeing the menstrua, e. g., by dissolving in them suitable dyestuffs. Or, a colored transparent coating may, if desired, be applied over the aluminum surface to change the color thereof.

As has been shown, the invention results in marked improvements in paper coated with aluminum powder deposited from aqueous suspensions. Improvements result in part from the novel composition of the coatings, and in part from finishing treatments not before given aluminum-coated papers. Coatings containing the relatively low ratio of adhesive to aluminum powder shown, that is, "slack-sized" coatings, are found to respond to calendering and especially to buffing operations in a manner quite different from previous aqueous coated aluminum papers. The preferred form of the invention comprising a flexible base having a mineral-coating and a top coating of aluminum and adhesive, suitably calendered and buffed, is so similar in appearance to metal foil that it may be considered as an imitation foil.

In an effort to provide exact measurement of the optical characteristics of my calendered (and of my calendered and buffed) metal-coated products, I have caused the latter to be studied from the standpoints of (1) specular gloss and (2) luminous apparent reflectance, each of which measurements affords means of scientific definition of the optical characteristics, as will be explained in the following:

A distinguishing quality possessed by polished metal and other very shiny surfaces is a relatively high specular gloss. The specular gloss of a surface may be readily determined by finding the apparent reflectance in the direction of mir-

ror reflection through an instrument aperture which is adapted to the type of surface being studied. The photometric device used, of course, is calibrated against a permanent standard of apparent reflectance. Several reflectometers are available for making such measurements. One suitable reflectometer for measuring specular gloss is described briefly in the Journal of the Optical Society of America, volume 27, page 225.

10 The sample in question may be illuminated at an angle of 45° to the normal and viewed at an angle of minus 45° to the normal using a reflectometer similar to that mentioned which has circular apertures giving an aperture sum of 15 about 18°.

If ordinary "casein metallics," comprising paper coated with aluminum powder and a water-soluble adhesive in the heretofore conventional ratio of adhesive to metal, are measured under 20 the conditions mentioned above, they are found to have a specular gloss of about 10 on a scale where a perfectly reflecting surface would show 100. On the other hand, paper coated according to the present disclosure and properly super- 25 calendered will, under the same conditions, exhibit a specular gloss of at least 25, and preferably a specular gloss of 30 and very advantageously about 35 or better. In case the product of this invention is buffed after being super- 30 calendered, it will be found to have a specular gloss of at least 45 and preferably has a specular gloss lying between 45 and 60 or even higher.

In specific tests, specular gloss measurements showed the following values:

|    |                                                                           |      |
|----|---------------------------------------------------------------------------|------|
| 35 | 1. Fine polished aluminum foil                                            | 70.0 |
|    | 2. Calendered and buffed product of the present invention                 | 55.2 |
|    | 3. Calendered but unbuffed product of the present invention               | 34.7 |
| 40 | 4. Unpolished aluminum foil                                               | 10.5 |
|    | 5. A "casein metallic" paper of commerce comprising aluminum powder       | 7.6  |
|    | 6. Another "casein metallic" paper of commerce comprising aluminum powder | 7.0  |
| 45 | 7. A "lacquer metallic" paper of commerce comprising aluminum powder      | 5.3  |
|    | 8. Polished white Vitrolite                                               | 5.4  |

Each of the above values represents the mean 50 of readings taken from a plurality of settings over a surface.

It is found in the case of very shiny surfaces, i. e., surfaces having a specular gloss of over 50, that considerable differences in measured specular gloss can exist without being particularly noticeable to the eye. On the other hand, in the case of less shiny surfaces, small differences in specular gloss attract quick attention. For example, a sample of the buffed product of the present invention was found to have a specular gloss of 55, while a sample of very high grade polished aluminum foil had a specular gloss of 70; nevertheless, the difference between the two from merely visual inspection was very slight. 60 On the other hand, however, the visible difference between sheets having specular gloss values of 10 and of 25 was very marked indeed.

The measurement of the luminous apparent reflectance is another test by which the products of this invention may be distinguished, and which affords a numerical definition of "metallic appearance." In making this test the surface is illuminated at an angle of 45° from the normal and is viewed at 0° from the normal, measurement being made with a Hunter "multi-

purpose reflectometer" (J. Opt. Soc. Am., vol. 27, p. 225, 1937). The scale of measurement is calibrated between a value "0" for the luminous apparent reflectance of a perfectly reflecting mirror, and a value of "100" for a prepared magnesium oxide surface.

On this scale, a very finely polished aluminum foil was found to have a value of .05 and an unpolished or "dull" aluminum foil was found to have a value of about .68. The supercalendered and buffed metallic-coated paper of this invention has a value lying between .10 and .05 or less—e. g., about .08—while the calendered but unbuffed paper product has a value lying between .20 and about .15, or even less. Tested in this same manner, "standard" "casein-metallic" papers (aluminum) showed values of about .35 to about .30, while a "lacquer metallic" paper of commerce showed a value of about .24.

In determining numerical values of apparent reflectance contrast,  $C_r$ , the formula employed is

$$C_r = \frac{A(45^\circ, -45^\circ)}{A(45^\circ, 0^\circ)}$$

which formula recites the ratio of specular gloss to luminous apparent reflectance of the subject of the latter two tests. The measurements may be taken with the Hunter "multipurpose reflectometer" previously referred to, or a McNicholas "goniophotometer" (see Jour. of Research of the U. S. Bureau of Standards, vol. 13, page 211), employing a "photox" cell and approximately the same total source and receptor spreads as are employed with the Hunter instrument (e. g., about  $18^\circ$  in both the plane of the measuring light beams and the plane perpendicular thereto). Since the " $C_r$ " numerical values are large numbers, it may be preferable to cite the values in terms of  $\log_{10}C_r$ .

In specific tests apparent reflectance contrast values were found in accordance with the data of the following table, in which samples 1 through 7 were the same as samples 1 through 7 of the data above relative to specular gross measurements, "10" is another sample of the same material as "3" but made at a different time, and "11" is the calendered and buffed product of the present invention closely similar to sample 2 above but differing from the latter in that sample 11 was machine buffed whereas sample 2 was hand buffed:

| Sample | Apparent reflectance contrast, $C_r$ |                                       | Log $\log_{10}C_r$ |          |               |
|--------|--------------------------------------|---------------------------------------|--------------------|----------|---------------|
|        | Plane of beams parallel to grain     | Plane of beams perpendicular to grain | Mean               | Parallel | Perpendicular |
| 1      | 850                                  | 550                                   | 700                | 2.93     | 2.74          |
| 2      | 1,050                                | 330                                   | 690                | 3.02     | 2.52          |
| 3      | 140                                  | 125                                   | 133                | 2.15     | 2.10          |
| 4      | 10                                   | 72                                    | 41                 | 1.00     | 1.86          |
| 5      | 16.6                                 | 13.4                                  | 15                 | 1.22     | 1.13          |
| 6      | 16.1                                 | 14.7                                  | 15.4               | 1.21     | 1.17          |
| 7      | 13.7                                 | 11.2                                  | 12.5               | 1.14     | 1.05          |
| 10     | 360                                  | 310                                   | 335                | 2.56     | 2.49          |
| 11     | 990                                  | 340                                   | 665                | 3.00     | 2.63          |

In general, the calendered but unbuffed products of the present invention show average apparent reflectance contrast values upward from a minimum of 100 ( $\log_{10}C_r=2.00$ ), while the calendered and buffed products show average apparent reflectance contrast values upward from a minimum of 500 ( $\log_{10}C_r=2.70$ ).

It has been found that the products of the present invention have sufficiently low heat ray emissivity values to make them useful as heat insulating materials. Emissivity may be defined as the ratio between the quantity of heat radiated from the surface of a given body and the quantity which would be radiated by a theoretical, perfect black body of the same dimensions and at the same temperature, the emissivity of the black body being designated as unity. Polished aluminum foil is the accepted standard of excellence for reflective insulation. Any material having an emissivity of not over 0.15 may be considered excellent for insulation while anything with an emissivity of not over 0.2 is useful in insulating. Emissivities of over 0.2 in general are of little interest for reflective insulation.

The following table shows the normal emissivities of a number of materials, as determined with the surface at a temperature of  $212^\circ$  F., and the thermopile at normal room temperature:

|                                                                                              | Sample        | Emissivity           |
|----------------------------------------------------------------------------------------------|---------------|----------------------|
| 25                                                                                           | Aluminum foil | 0.045 (0.04 to 0.05) |
| A commercial heat-reflecting product consisting of sheet iron surfaced with a tin-lead alloy | 0.09          |                      |
| A sample of my calendered and buffed product                                                 | 0.09          |                      |
| A sample of my calendered product (not buffed)                                               | 0.12          |                      |
| Most prior reflective coated papers                                                          | 0.32 to 0.49  |                      |
| Majority of ordinary non-metallic materials                                                  | 0.85 to 0.95  |                      |
| 30 "Black body," perfect radiator                                                            | 1.00          |                      |

Generally speaking my calendered product, when measured under the conditions specified above, has an emissivity value of 0.2 or less, usually about 0.15 or less, and my buffed product has an emissivity value of about 0.1 or less.

Prior aluminum coated papers in which the metallic coating was substantially uniform throughout, e. g., coatings of either the casein-metallic or lacquer-metallic type, have surely not approached the low emissivity value of 0.2, much less the still lower value of 0.1. In fact it is to be doubted that any paper coated with aluminum powder has, prior to my invention, had the low emissivity value of 0.1.

It appears, therefore, that my product provides an entirely new kind of heat-insulating paper. It also provides a decorative paper having a degree of gloss not previously believed attainable in a casein-aluminum coated sheet. While very low emissivity and very high specular gloss are not necessarily correlated, they both may exist in the same sheet of my product.

While the invention has been described in relation to a coated paper it should be apparent that the coating described may equally well be applied to various other sheet materials without important changes in procedure, and will in those cases also result in aluminum-coated products having gloss and emissivity values not before attained by water-deposited aluminum coatings.

While the present invention is particularly concerned with the provision of metallic coated sheet material (e. g., metal foil-simulating metallic coated paper) wherein the metal is aluminum, it is fully within the scope of the invention to substitute, wholly or in part, finely divided copper, or finely divided copper alloy, in flake form, for the aluminum powder above described. In such event, one adheres to the concept of employing a less than conventional adhesive-to-metal powder weight ratio.

This application is a continuation-in-part of co-pending Serial No. 284,089, filed July 12, 1939.

I claim:

Process of making an aluminum coated paper product simulating aluminum foil, which comprises coating a paper base with a mineral coating composition and calendering the coated paper base, applying to and spreading over the mineral coated and calendered paper base a layer of aqueous aluminum powder-containing coating composition containing substantially greaseless aluminum powder, a wetting agent for dispersing the aluminum powder and a water-dispersible

protein adhesive, the weight ratio of adhesive to aluminum being from 15 to 35 parts adhesive to 100 parts aluminum, the layer of aluminum coating composition being of a thickness to add, when dried, from 1 to not more than 5 pounds of the adhesive-aluminum composition per ream to the weight of the paper, drying the coating, moistening the surface of the dried aluminum coated paper, and severely supercalendering the latter.

JOHN W. CLARK.